

## UNITED STATES PATENT OFFICE

2,359,063

## LUBRICATING OIL

Paul R. Van Ess, Berkeley, Calif., assignor to Shell Development Company, San Francisco, Calif., a corporation of Delaware

No Drawing. Application September 23, 1941,  
Serial No. 411,972

17 Claims. (Cl. 252—33)

This invention relates to improved lubricating oils, and more particularly is concerned with compounded mineral lubricating oils to which have been added small amounts of certain organic arsine disulfides.

It is already known that the presence of various sulfur and arsenic compounds in lubricating oils may exert beneficial influences. Thus sulfur compounds have been added in order to increase the load-carrying capacity of the oil, or to retard corrosion toward certain alloy bearing metals, etc. Arsenic compounds have been used to improve oiliness, to retard corrosion and to reduce wear.

The effect of sulfur in particular as an anti-corrosive has been in the past a subject of considerable investigation, and it has been found that different sulfur compounds are widely different in their effect. Many sulfur compounds, such as thiophenes, are wholly ineffective. Others are so extremely active that they frequently induce corrosion, particularly to ferrous metals. For example, free sulfur,  $H_2S$  or compounds readily liberating S or  $H_2S$ , while protecting certain alloys, are very dangerous, particularly when used in the lubrication of internal combustion engines. It thus appears that the sulfur in the compound must possess an activity toward bearing metals above a certain minimum in order to display its protective effect, and, on the other hand, it must not be so active as to cause corrosion to ferrous metals.

The problem of relative corrosiveness or anti-corrosiveness of various compounds is further complicated by the fact that lubricating oils containing them are used over wide temperature ranges and under hydrolyzing and/or oxidizing conditions. In the past, the influence of these factors has not been sufficiently taken into consideration, and therefore much of the information available is contradictory and misleading.

The ideal anti-corrosion compound is one which is readily soluble in hydrocarbon oils and which over a wide temperature range, i. e., from about normal room temperature up to about 200° C. (the highest crank case temperature likely ever to be encountered) is sufficiently active to prevent or retard corrosion of bearing metals, and, on the other hand, is not so active as to attack ferrous metals within the same temperature range.

Among the many additives for lubricating oils is triphenyl arsine sulfide which, although useful, unfortunately has a limited solubility in lubricating oils, it being, in general, impossible

to dissolve more than .1 to .2% without danger of precipitating at least a portion thereof.

It is a purpose of this invention to produce a lubricating oil suitable for internal combustion engines which is non-corrosive to bearing metals over the entire normal temperature range of internal combustion engines. It is another purpose to produce a compounded non-corrosive lubricating oil containing dissolved a detergent which under normal lubricating conditions may induce corrosion and in addition a relatively large amount of an arsine sulfide. A further purpose is to produce a lubricant which materially reduces wear under hydrolyzing and/or oxidizing conditions. Still another purpose is to produce a lubricating oil containing an arsenic compound which is easy to manufacture, is readily soluble in hydrocarbon oils in quantities above about .1%, is substantially non-volatile and which, even at elevated temperatures, does not have the repulsive odor possessed by many organic arsenic compounds.

I have discovered that lubricating oils to which have been added small amounts of organic arsine disulfides possessing the formula



wherein R is a hydrocarbon radical having at least 4 carbon atoms, have the desired anti-corrosive properties for bearing alloys over the entire normal crankcase temperature range and over prolonged operating conditions, as may occur in internal combustion engines. The arsine disulfides of this invention are oil-soluble in useful quantities, stable and non-volatile, and the sulfur in them does not attack ferrous metals even at elevated temperatures.

The hydrocarbon radical may be aliphatic, alicyclic or aliphatic substituted aromatic, aliphatic chains being preferred, particularly those having 10 or more carbon atoms, for reasons discussed later. It may contain polar substitution radicals provided that they do not unduly limit the oil-solubility of the compound. Thus it may contain hydroxyl, ether, sulfide, amino, imino, halogen, etc., radicals.

Suitable unsubstituted hydrocarbon radicals are, for example, butyl, isobutyl, tertiary butyl, primary, secondary or tertiary amyl, hexyl, cyclohexyl, heptyl, methyl cyclohexyl, octyl, iso-octyl, decyl, cetyl, various naphthenyl, naphthyl, methyl naphthyl, butyl naphthyl, wax phenyl, wax naphthyl, wax anthracyl, phenyl- or naphthyl-, -methylene, -ethylene, -cetylene, etc. The amounts of arsine disulfides required to

suppress corrosion vary normally between about 0.05-2% and preferably between 0.2-0.5%.

As is known, compounds of certain elements, among which are phosphorus, arsenic and antimony, may, under certain conditions, reduce wear experienced under normal lubricating conditions. This reduction has been traced to the formation of low-melting alloys of the elements with submicroscopic high spots of the metal surface which is being lubricated. Because of the relatively low melting point of the alloy, the high spot melts away and fills in minute depressions, thereby causing an effective polishing of the bearing surface without the use of an abrasive. On the perfectly smooth bearing surface, the load is more evenly distributed which results in more perfect fluid lubrication and reduces the wear. The presence of certain polar compounds having long carbon chains further enhances the wear reduction by forming wedges between the gliding metal surfaces.

It has been shown, however, that certain disturbing influences may completely destroy any advantages that may possibly be gained by the addition of "chemical polishing compounds." For example, under conditions favoring corrosion, the polishing may be offset by the corrosion, newly formed high spots being continuously formed which are then melted down. As a result, the rate of wear may increase rather than decrease. Such has been found to be the case, for example, with tricresyl phosphate which, when tested in the so-called four-ball machine (described in "Engineering," vol. 136 (1938) p. 46) proves to be an excellent anti-wear agent, but in an internal combustion engine actually increases wear. In the latter case, apparently, traces of phosphoric acids are liberated, probably due to hydrolysis, which traces are responsible for corrosion resulting in increased wear by the mechanism explained above.

Moreover, the formation of the alloy in the polishing mechanism requires that the alloy-forming element can be liberated at the proper moment. Oxidized compounds of the elements must first be reduced before the element can be freed, and it was found that for this reason, in general, oxidized compounds are poorer polishing agents than non-oxidized ones. For example, an arsine is a better polishing compound than an arsenite or arsenate.

Arsine disulfides in which the organic radical contains arsenic, hydrocarbon chains of 10 or more carbon atoms have the advantage of being able to produce the wedging effect mentioned earlier, thereby further reducing wear. Thus these compounds combine the three properties of highly effective corrosion protection under a wide range of conditions, effective chemical polishing and wear-reducing due to wedging effect.

The arsine disulfides of this invention are particularly useful for the purpose of suppressing the corrosiveness of lubricating oils containing added small amounts of detergents, e. g., from .25%-5% of detergents, such as the oil-soluble salts of polyvalent metals or organic amines with detergent-forming acids, for example, naphthenic, aromatic carboxylic, paraffin carboxylic, rosin, petroleum sulfonic, alkyl aromatic, sulfonic, etc., acids, voltolized fatty or mineral oils, voltolized paraffin wax, polymers obtained by polymerization of unsaturated fatty oils with  $BF_3$ , etc.

Arsine disulfides can be produced, for example, by reacting arsenous oxide; i. e.,  $As_2O_3$ , with an alcohol having at least 4 carbon atoms in the

presence of air to produce an arsine dioxide in accordance with the formula:



5 The arsine dioxide is then dissolved in water or some other suitable solvent, such as an aqueous lower alcohol, and into the resulting solution  $H_2S$  is bubbled. Arsine disulfide is precipitated as a pasty or oily mass which is separated and dried.

10 The dry product is readily soluble in hydrocarbon oils.

The following examples further illustrate my invention:

#### EXAMPLE I

15 55 V. I. lubricating oil S. A. E. 30 grade was divided into two portions. To one portion was added 1.25% by weight of calcium petroleum sulfonate. This doped portion was subdivided into two portions and to one of these portions was added .2% of normal butyl arsine disulfide.

20 The doped and undoped oils were then tested by a test known as the Thrust bearing corrosion test, which is carried out as follows: A hardened steel disc is made to rotate for 20 hours under constant pressure against three flat copper-lead bearings. The bearing assembly rests in a steel cup filled with the oil to be tested, and the temperature of the oil maintained at a predetermined figure by thermostatic control. The bearings are weighed before and after the test, the difference in weight representing the loss sustained during the test. The tests were run with the same bearings and oil until the end of the last recorded period. Intermediate bearing losses were determined by removing, cleaning, and weighing the bearings and then placing them back in the machine to continue the test. Results were as follows:

40

Table I

| Oil         | Additive                                                    | Bearing wgt. loss in mg./sq. cm. at 120° C. |                                                           |
|-------------|-------------------------------------------------------------|---------------------------------------------|-----------------------------------------------------------|
|             |                                                             | 1st 20 hours                                | 2nd 20 hours                                              |
| S. A. E. 30 | None                                                        | 2                                           | 2                                                         |
| S. A. E. 30 | Calcium petroleum sulfonate.                                | 17.5                                        | Overheated because of excessive corrosion and roughening. |
| S. A. E. 30 | Calcium petroleum sulfonate + .1% n-butyl-arsine disulfide. | 0.2                                         | 0.1                                                       |

55 The test results of Table I indicate that the corrosivity of the calcium petroleum sulfonate has been substantially eliminated by the butyl arsine disulfide.

#### EXAMPLE II

60 A voltolized oil was prepared by subjecting a rape-seed oil having a viscosity of 236 S. U. Secs. at 100° F. and 60.5 S. U. Secs. at 210° F. (V. I. 154) to silent electrical discharges for 4 hours at 210° F., at which time it possessed the following characteristics: Viscosity 3402 S. U. Secs. at 100° F. and 392 S. U. Secs. at 210° F., and V. I. 128. To a 55 V. I. lubricating oil, S. A. E. 30 grade, was added .9% by weight of this voltolized rapeseed oil. This dope was subdivided into two portions and to one of these portions was added .1% by weight of normal butyl arsine disulfide. The doped and undoped oils were then tested in a Lauson engine, which

65 is a 4-cycle, L-head vertical single cylinder engine. Oil is circulated through the engine by a pump which takes suction on an oil reservoir.

The crankcase oil temperature of 100° C. is controlled by a strip heater mounted under the crankcase. The jacket temperature is maintained at 140° C. by an evaporative cooling system. The engine is run at 1700 R. P. M. for 30 hours. New copper-lead bearing shells are placed in the connecting rod before each test.

Results were as follows:

Table II

| Oil         | Additive agent                                             | Bearing loss in mg./half bearing |               |
|-------------|------------------------------------------------------------|----------------------------------|---------------|
|             |                                                            | Upper bearing                    | Lower bearing |
| S. A. E. 30 | .9% voltolized rapeseed oil                                | 19.2                             | 4.8           |
| S. A. E. 30 | .9% voltolized rapeseed oil + .1% n-butyl arsine disulfide | 6.6                              | 0.2           |

EXAMPLE III

A 55 V. I. lubricating oil, S. A. E. 30 grade, containing 1.25% of calcium petroleum sulfonate was run in a Caterpillar Diesel engine for 60 hours. The oil was too corrosive at this stage to be tested by the Thrust bearing corrosion test, described in Example I. .2% by weight of n-butyl arsine disulfide was added to the used oil and this doped-used oil subjected to the Thrust bearing corrosion test at 107° C. for 20 hours, using copper-lead bearings. The bearings tested in the doped-used oil showed no measurable loss of weight, indicating the corrosivity of the oil was substantially completely overcome by the addition of the n-butyl arsine disulfide.

I claim as my invention:

1. A non-corrosive lubricating oil comprising a predominant amount of a mineral lubricating oil containing dissolved a small amount of an oil-soluble arsine disulfide having the formula  $RAsS_2$ , wherein R is a hydrocarbon radical having at least 4 aliphatic carbon atoms.

2. A non-corrosive lubricating oil comprising a predominant amount of a mineral lubricating oil containing dissolved a small amount of an oil-soluble arsine disulfide having the formula  $RAsS_2$ , wherein R is an aliphatic hydrocarbon radical having at least 10 carbon atoms.

3. A non-corrosive lubricating oil comprising a predominant amount of a mineral lubricating oil containing dissolved between 0.05-2% of an oil-soluble arsine disulfide having the formula  $RAsS_2$ , wherein R is a hydrocarbon radical having at least 4 aliphatic carbon atoms.

4. A non-corrosive mineral lubricating oil containing an added oil-soluble detergent normally causing corrosion and a small amount of an arsine disulfide having the formula  $RAsS_2$ , wherein R is a hydrocarbon radical having at least 4 aliphatic carbon atoms the amount of said disulfide being sufficient to reduce the corrosiveness of said added detergent.

5. A non-corrosive mineral lubricating oil containing dissolved from .25% to 5% of a salt of a polyvalent metal with a detergent-forming acid and from 0.05% to 2% arsine disulfide having the formula  $RAsS_2$ , wherein R is a hydrocarbon radical having at least 4 aliphatic carbon atoms.

6. A non-corrosive mineral lubricating oil containing a corrosion-inducing amount of a

high molecular weight hydrocarbon polymer having detergent properties and a small amount of an arsine disulfide having the formula  $RAsS_2$ , wherein R is a hydrocarbon radical having at least 4 aliphatic carbon atoms.

7. A non-corrosive mineral lubricating oil containing a corrosion-inducing amount of a voltolized oleaginous substance and a small amount of an arsine disulfide having the formula  $RAsS_2$ , wherein R is a hydrocarbon radical having at least 4 aliphatic carbon atoms.

8. A non-corrosive mineral lubricating oil containing a corrosion-inducing amount of a voltolized rapeseed oil and a small amount of an arsine disulfide having the formula  $RAsS_2$ , wherein R is a hydrocarbon radical having at least 4 aliphatic carbon atoms.

9. The composition of claim 1, wherein the arsine disulfide is normal butyl arsine disulfide.

10. A method of lubricating alloy bearings of the group consisting of copper and lead alloy bearings in internal combustion engines which method consists in applying to the bearing surfaces a non-corrosive compounded lubricating oil comprising a predominant amount of a mineral lubricating oil which contains (1) an amount of an oil-soluble detergent normally sufficient to impart corrosive properties to said oil and (2) an amount of an oil-soluble arsine disulfide having the formula  $RAsS_2$  wherein R is a hydrocarbon radical having at least 4 aliphatic carbon atoms, which amount of arsine disulfide is sufficient to render said corrosive oil substantially non-corrosive.

11. The method of claim 10 wherein the detergent is calcium petroleum sulfonate.

12. The method of claim 10 wherein the detergent is calcium petroleum sulfonate and the disulfide is n-butyl arsine disulfide.

13. A method of lubricating alloy bearings of the group consisting of copper and lead alloy bearings in internal combustion engines which method consists in applying to the bearing surfaces the composition of claim 1, thereby inhibiting corrosion of the bearing surface.

14. A method of lubricating alloy bearings of the group consisting of copper and lead alloy bearings in internal combustion engines which method consists in applying to the bearing surfaces the composition of claim 5, thereby inhibiting corrosion of the bearing surface.

15. A method of lubricating alloy bearings of the group consisting of copper and lead alloy bearings in internal combustion engines which method consists in applying to the bearing surfaces the composition of claim 6, thereby inhibiting corrosion of the bearing surface.

16. A method of lubricating alloy bearings of the group consisting of copper and lead alloy bearings in internal combustion engines which method consists in applying to the bearing surfaces the composition of claim 7, thereby inhibiting corrosion of the bearing surface.

17. A method of lubricating alloy bearings of the group consisting of copper and lead alloy bearings in internal combustion engines which method consists in applying to the bearing surfaces the composition of claim 8, thereby inhibiting corrosion of the bearing surface.

PAUL R. VAN ESS.